

July 11, 1950

C. MACK  
PROCESS FOR THE REGENERATION  
OF DESULFURIZING CATALYST  
Filed Oct. 25, 1947

2,515,131



Charles Mack Inventor

By W. O. T. Filman attorney

## UNITED STATES PATENT OFFICE

2,515,131

PROCESS FOR THE REGENERATION OF  
DESULFURIZING CATALYSTCharles Mack, Sarnia, Ontario, Canada, assignor  
to Standard Oil Development Company, a cor-  
poration of Delaware

Application October 25, 1947, Serial No. 782,125

5 Claims. (Cl. 196—28)

1

The present invention is concerned with the desulphurization of oils. The invention is especially directed to the regeneration of catalysts such as bauxite which are utilized in the desulphurization of petroleum oils, particularly those boiling in the motor fuel boiling range. In accordance with the present process, spent bauxite catalyst employed in the desulphurization of oils is more fully and completely regenerated by a two stage regeneration operation which comprises a burning stage and an ammonia treating stage.

It is known in the art to desulphurize petroleum oils by contacting feed oils with bauxite at elevated temperatures by various processes. For example, it is known to remove objectionable sulphur compounds from virgin feed oils by contacting the same with bauxite at temperatures in the range of from about 600° F. to 650° F. It is also known to treat distillates boiling in the motor fuel boiling range secured from various cracking operations with bauxite at temperatures in the range from about 600° F. to 900° F., usually in the range from about 600° F. to 800° F. The pressures employed in the desulphurization operation may be atmospheric or as high as 300 to 400 pounds per square inch gauge. These petroleum oils boiling in the range from about 100° F. to 420° F. may be treated in the vapor or liquid phase depending upon the pressure. In general the oils are contacted with bauxite under non-cracking conditions. Under these conditions substantially no change of molecular weight and boiling range results and very little fixed gas is evolved other than hydrogen. The bauxite catalyst is then usually regenerated by burning at temperatures in the range from about 1100° F. to 1300° F. and higher.

In these desulphurization operations, commercial bauxites are utilized which contain various concentrations of iron oxides as impurities. For example, the concentration of iron oxide may vary from as low as 0.5% to as high as 25% by weight based upon the alumina. One conventional procedure for the manufacture of a low iron content bauxite is to treat a natural bauxite containing 4% to 5% iron oxide at a temperature of about 1000° F. This changes the iron to a magnetic form. The iron is then removed by means of a magnetic separator. By this treatment the iron oxide content of the treated bauxite is reduced to about 2½% to 3%.

Also, in these desulphurization operations, the sulphur compounds which usually comprise mercaptans and organic sulphides tend to break down

2

to form hydrogen sulphide at the above-mentioned temperature range. While the aluminum oxide in the bauxite does not react with the hydrogen sulphide at a temperature in the range from 600 to 900° F., the iron oxide present does react with the hydrogen sulphide resulting in the production of the metal sulphide. Thus, upon regeneration of the catalyst by burning off the carbonaceous material with air at a temperature in the range from about 1100° F. to 1300° F. oxidation of the iron sulphide to the corresponding sulphite and sulphate will result. At high temperatures, as for example, 900° F. and above, the sulphite and sulphate will partly disassociate to sulphur dioxide and iron sulphide and part of these constituents will be retained on the catalyst. Upon subsequent use of the regenerated catalyst the hydrogen sulphide formed from the break down of the sulphur compounds as described will react with the sulphur dioxide generated on the catalyst to form free sulphur which will contaminate the hydrocarbons being desulphurized.

I have now discovered a process which will substantially overcome this difficulty. My process comprises regenerating spent bauxites utilized in the desulphurization of petroleum oils by a two stage process. In the initial stage I burn the carbonaceous materials at elevated temperatures and in the secondary stage I treat the burnt bauxite with ammonia, preferably at elevated temperatures.

The process of my invention may be readily understood by reference to the drawing illustrating one embodiment of the same. Referring specifically to the drawing, a petroleum oil containing undesirable sulphur compounds is introduced into treating zone 1 by means of feed line 10. Zone 1 contains a bauxite treating agent which contains as an impurity iron oxide. The treated oil substantially free of undesirable sulphur compounds is withdrawn from treating zone 1 by means of line 11. After the bauxite has become spent so that it will not reduce or remove the sulphur compounds from the oil being treated to the desired degree, the feed oil is then introduced into zone 2 by means of line 12. Zone 2 is equivalent to zone 1 and no attempt will be made to describe the operation of zone 2 in detail. The treated oil is withdrawn from zone 2 by means of line 13 and withdrawn from the system by means of line 14. The spent bauxite in zone 1 is treated by introducing air or other oxygen containing gas by means of line 14 in order to burn off the carbonaceous material.

## 3

The combustion gases are removed from zone 1 by means of line 15. I then purge the bauxite by means of an inert gas, which is preferably nitrogen, which is introduced into zone 1 by means of line 16 and withdrawn by means of line 15. Then, in accordance with my process I introduce ammonia into zone 1 by means of line 17 and withdraw the same by means of line 18. This stream may be handled in any manner desirable, as for example, it may be recycled or purified as desired. After the bauxite in zone 1 has been regenerated and the bauxite in zone 2 has become spent so that it will not satisfactorily remove sulphur compounds from the oil being treated, the feed oil stream is then reintroduced into zone 1 and the bauxite in zone 2 is regenerated as hereinbefore described.

My process comprises a two stage method for the regeneration of spent bauxite. In accordance with my process, I have found that the formation of free sulphur is eliminated, if after burning off of the carbonaceous deposits, the catalyst is treated at an elevated temperature with ammonia. During this stage, the iron sulphite and sulphate are converted into the corresponding ammonium salts which are volatile at high temperatures.

In order to further illustrate my process, the following example is given illustrating one embodiment of the same:

*Example*

A plant sample of bauxite which had been repeatedly regenerated at 1200° F. in a stream of air showed the presence of iron sulphite and sulphate equivalent to 2% of  $\text{SO}_4$ . This bauxite was utilized in the treatment of a naphtha boiling in the range from about 100° F. to 420° F. The naphtha was also treated with fresh bauxite. Another sample of a naphtha was treated with the regenerated bauxite except that in this latter treatment the regenerated bauxite was regenerated in accordance with my process wherein the bauxite was contacted with ammonia at 800° F. The three desulphurization operations were carried out at 800° F. The naphtha treated contained normal butyl mercaptan in an amount of 0.27% equivalent to 0.1% of sulphur. The mixture was found to pass the copper strip test.

The results obtained are as follows:

| Catalyst                                 | Copper Strip Test <sup>1</sup> on Naphtha | Mercaptans in Naphtha |
|------------------------------------------|-------------------------------------------|-----------------------|
| Fresh Bauxite                            | Pass                                      | None                  |
| Regenerated Bauxite                      | Does not pass                             | Do.                   |
| Regenerated Bauxite treated with Ammonia | Pass                                      | Do.                   |

<sup>1</sup> A. S. T. M. Designation D849-45T.

My invention specifically applies to desulphurization operations wherein petroleum oils boiling in the motor fuel boiling range are treated in the vapor phase under non-cracking conditions utilizing bauxites at temperatures in the range from about 600° F. to 900° F. It is particularly adapted to those bauxites containing from 0.5 to 10%  $\text{Fe}_2\text{O}_3$  as an impurity. It is especially adapted for the regeneration of bauxites containing in excess of 3%  $\text{Fe}_2\text{O}_3$  as an impurity. The temperature used in the burning or initial stage may be any satisfactory temperature, but generally is in the range from about 1000° F. to 1300° F.

## 4

The temperature employed in the secondary stage, or ammonia treating stage, is preferably in the range from 600° F. to 900° F. It is very desirable that this ammonia treating operation be conducted in an inert atmosphere, preferably in an atmosphere of nitrogen or flue gas.

I claim:

1. Improved process for the removal of mercaptans and organic sulphides from petroleum oils boiling in the gasoline boiling range which comprises contacting said oils with bauxite containing iron oxide as an impurity at a temperature in the range from about 600° F. to 900° F., removing said bauxite from the feed oil after the same has become spent to the extent that the bauxite will not satisfactorily remove said mercaptans from the oil to the desired extent, burning said bauxite with an oxygen containing gas at a temperature in the range from about 1000° F. to 1400° F., placing said burned bauxite in an inert atmosphere and treating the same with ammonia in a secondary stage, removing said ammonia and again contacting the bauxite with feed oil containing mercaptans.
2. Process as defined by claim 1 wherein the temperature employed when treating said bauxite with ammonia is in the range from about 600° F. to 900° F.
3. Process as defined by claim 2 wherein the concentration of the iron oxide ( $\text{Fe}_2\text{O}_3$ ) in said bauxite is in the range from about 3% to 10%.
4. Improved process for the regeneration of bauxite containing more than about 3% of iron oxide as an impurity, said bauxite having been employed in the desulphurization of oils which comprises burning the bauxite in an initial stage at a temperature in the range of about 600 to 900° F., followed by treating the burned bauxite with ammonia in a secondary stage at a temperature in the range from about 600° F. to 900° F.
5. The process defined by claim 4 wherein the bauxite is treated with ammonia in a secondary stage in an inert atmosphere at a temperature of about 800° F.

CHARLES MACK.

## REFERENCES CITED

The following references are of record in the file of this patent:

## UNITED STATES PATENTS

| Number    | Name            | Date          |
|-----------|-----------------|---------------|
| 2,016,271 | Buell et al.    | Oct. 8, 1935  |
| 2,160,874 | Kinsel          | June 6, 1939  |
| 2,162,319 | Schulze         | June 13, 1939 |
| 2,225,782 | Ipatieff et al. | Dec. 24, 1940 |
| 2,225,811 | Wells           | Dec. 24, 1940 |
| 2,242,387 | Boyd            | May 20, 1941  |
| 2,267,735 | Ipatieff et al. | Dec. 30, 1941 |
| 2,326,369 | La Lande        | Aug. 10, 1943 |
| 2,331,343 | Phillips        | Oct. 12, 1943 |
| 2,412,868 | Brown           | Dec. 17, 1946 |

## FOREIGN PATENTS

| Number  | Country       | Date          |
|---------|---------------|---------------|
| 337,348 | Great Britain | Oct. 23, 1930 |

## OTHER REFERENCES

Helmers et al., "Catalytic Desulfurization . . . Over Bauxite," Petroleum Processing, Feb., 1948, 70 pages 133 to 138.